

No. 792,638.

PATENTED JUNE 20, 1905.

W. R. WHITNEY.

ARTIFICIAL RESISTANCE.

APPLICATION FILED NOV. 16, 1901. RENEWED NOV. 3, 1904.

Fig.1.



Fig. 2.



Witnesses

J. Ellis Glenn.

Benjamin B. Hule.

Inventor

Willis R. Whitney.

by Albert S. Davis  
Atty.

## UNITED STATES PATENT OFFICE.

WILLIS R. WHITNEY, OF BOSTON, MASSACHUSETTS, ASSIGNOR TO GENERAL ELECTRIC COMPANY, A CORPORATION OF NEW YORK.

## ARTIFICIAL RESISTANCE.

SPECIFICATION forming part of Letters Patent No. 792,638, dated June 20, 1905.

Application filed November 16, 1901. Renewed November 3, 1904. Serial No. 231,205.

*To all whom it may concern:*

Be it known that I, WILLIS R. WHITNEY, a citizen of the United States, residing at Boston, in the county of Suffolk, State of Massachusetts, have invented certain new and useful Improvements in Artificial Resistances, of which the following is a specification.

Electrical resistances are frequently formed of mixtures of graphite, carbon-dust, or other conducting material with some binding substance, such as ordinary clay or the constituents of which porcelain is made. The substances chosen are formed while in a plastic state into the desired shapes and are then dried and baked. Such artificial resistances, usually in the form of rods, are largely used in the construction of lightning-arresters, as resistances for electrical measuring instruments, &c. In many cases it is desirable to produce large numbers of these resistance devices each of the same size and shape, composition, and resistance. It has been found in practice, however, that even though the composition of the resistance devices, such as rods, be as nearly as possible the same in all the rods the resistances of the rods will vary very greatly. Thus, for example, some of the rods, which are to all appearances identical with others, may differ in resistance by fifty or seventy-five per cent., or even much more. I have discovered that in resistance-bodies of the character mentioned the conductivity, such as it is, often resides very largely in the surface coating or skin of the body and that if this surface be removed, even to the depth of only a few thousandths of an inch, the conductivity of the body as a whole is largely reduced or, which is the same thing, the resistance increased. The important fact, however, is that when a large number of these resistance-bodies which differ largely in resistance among themselves are treated in the manner described the resistances of the bodies become almost uniform. I have discovered that the same result may be secured in a variety of ways—such, for example, as by removing the exterior surface of the resistance devices by abrasion or by the application of heat. By the latter method, which I consider preferable, the re-

sistance-body is exposed to an intense heat in 50 the presence of air. The conducting material on the surface of the body is thereby burned away, leaving the binding substance in the form of baked clay or porcelain. The depth to which the conducting substance is burned 55 away may be varied by varying the length of heating of the resistance-body, as will be evident.

By the application of this method resistance-bodies, such as pencils, may be made in large 60 quantities and all of substantially uniform resistance. If desired, the exposed layer of baked clay or porcelain forming the outside of the resistance-pencils may be covered with a glaze. Whether or not a glaze is used, the 65 outer surface of the resistance device, being more or less vitrified, furnishes a good protection against dampness, and so tends to preserve a uniform resistance of the device.

The novel features which characterize my 70 invention I have set forth with particularity in the appended claims.

For a detailed description of my invention reference is to be had to the following specification, taken in connection with the accompanying drawings, in which—

Figure 1 represents one of the many utilities of which my invention is capable, and Fig. 2 is a perspective view of a resistance-pencil made in accordance with my invention. 80

Fig. 1 represents a lightning-arrester of well-known type in which the current-limiting resistance 1 is constructed in accordance with my invention.

Fig. 2 represents in detail the resistance device shown in Fig. 1. This device will be seen to consist of a pencil 1, having an outer coating 2 and an interior portion shown in section at 3. The pencil is constructed by molding the same from a plastic mixture of 90 clay or other earthy non-conducting or at least poorly-conducting material with a minor proportion of some conducting material, such as graphite, powdered carbon, carborundum, or the like. Of the conducting substances 95 mentioned I much prefer to use carborundum, since it more easily produces homogeneous resistance material, due to the fact that

a larger proportion of the same may be used than of graphite and also due to the fact that it may be obtained in an impalpable powder, while graphite is always more or less flaky.

5 After the rods or other resistance devices have been formed from the resistance material while in the plastic condition they are dried and then heated or burned, as above described, in an electric resistance - muffle or other furnace until the conducting substance is burned away from the surface, leaving an outer coating of more or less vitreous non-conducting substance. If desired, the rods may be baked preliminary to the burning off 15 of the outer surface of conducting substance.

To make electrical connection with the conducting material of the pencil when thus treated by heat, various means may be employed. Thus the non-conducting surface may be removed and contact made with the exposed conducting portion. This is shown clearly in Fig. 2, in which the left-hand end 4 of the rod is cut away sufficiently to expose a cylindrical surface of conducting interior. If desired, the extreme end of the rod might be cut or broken off and contact then made with the exposed circular section of conducting material. In any case the contact I find may be much improved by applying a metal coating 30 to the contact-surface. I do this by rubbing the surface with a soft metal, such as lead, which by abrasive action of the surface is deposited in the pores and forms a smooth adherent good-conducting coating. The surface, if cylindrical, may be revolved against the soft metal in a lathe or otherwise. A surface thus treated is intended to be represented at 4.

It has been found in practice that in lightning-arresters making use of the ordinary resistance-rods the resistance of the rods after 40 a discharge has passed may be so much higher as to make the device useless so far as any further protection is concerned. This may be due to the action of heat generated in the rods in driving away moisture which may be present in the rods, or the heat may be sufficiently intense to cause more or less oxidation and wasting away of the carbon or other conducting material present in relatively high 45 percentage in the outer skin of the rods. Rods made in accordance with my invention are not subject to this disadvantage. Being provided with a weatherproof coating, they are not affected by moisture, and having no outer skin of relatively high conductivity they 50 are not subject to permanent alteration of conductivity by heat.

What I claim as new, and desire to secure by Letters Patent of the United States, is—  
60 1. The method of producing artificial resistances which consists in combining a conduct-

ing substance such as carborundum with a binding material such as clay, then baking the resistance device and subsequently burning away the outer surface of conducting mate- 65 rial.

2. The method of equalizing the specific resistances of a plurality of resistance devices formed of a mixture of a conducting and a non-conducting material which consists in removing the surface coating of conducting material. 70

3. The method of producing artificial resistances which consists in combining a conducting substance with a non-conducting binding 75 material, forming the resultant mass while in a plastic state into the shape desired, drying the same and subsequently burning away the conducting material contained in the exposed surface of the device. 80

4. The method of making contact with a porous resistance-body which consists in mechanically filling the pores of a selected portion of the surface of said body with some soft metal and applying a terminal to the surface thus 85 treated.

5. The method of producing artificial resistances which consists in combining a conducting substance such as carborundum with a non-conducting binding material such as clay, 90 molding the material while plastic, then drying, and burning away the conducting material in the outer surface of the devices thus molded.

6. The method of producing an artificial 95 high-resistance body, which consists in combining a conducting substance with a relatively non-conducting binding material, molding the material while plastic, baking, and mechanically filling the pores of a selected portion of the surface of the body with some soft metal. 100

7. The method of applying a conducting coating to a porous resistance-body, which consists in filling the pores of a selected portion of the surface of the body with metal by 105 abrasive action between the body and a body of the metal selected.

8. The method of applying a good electrically-conducting contact-surface to a body of porous or earthy material, which consists in producing an abrasive action between the body and a mass or body of metal thereby causing a deposit of metal in the pores of that portion of the surface of said body of porous or earthy material submitted to such abrasive 115 action.

In witness whereof I have hereunto set my hand this 15th day of November, 1901.

WILLIS R. WHITNEY.

Witnesses:

BENJAMIN B. HULL,  
HELEN ORFORD.